

# UNITED STATES PATENT OFFICE.

JOHN C. BAKER, OF RIDGEFIELD PARK, NEW JERSEY, ASSIGNOR TO WALLACE & TIERMAN CO. INC., OF BELLEVILLE, NEW JERSEY, A CORPORATION OF NEW YORK.

## PROCESS OF BLEACHING PAPER AND FABRICS.

1,413,154.

Specification of Letters Patent. Patented Apr. 18, 1922.

No Drawing.

Application filed July 18, 1921. Serial No. 485,701.

*To all whom it may concern:*

Be it known that I, JOHN CLARK BAKER, a citizen of the United States of America, residing at Ridgefield Park, county of Bergen, and State of New Jersey, have invented certain new and useful Improvements in Processes of Bleaching Paper and Fabrics, of which the following is a full, clear, and exact description.

10 The invention, subject of my present application for Letters Patent, is a new and improved process of bleaching such materials as the fibres of paper pulp, and for a clear understanding of its nature, a brief 15 review of the methods heretofore followed in such cases is apposite.

In one method which has been practiced in this art, the result has been largely accomplished by subjecting the fibres in the 20 form of pulp to the action of an aqueous solution of bleaching powder, which is composed essentially of calcium hypochlorite containing varying amounts of dissolved calcium hydroxide. These and like solutions, however, are notably slow in their 25 bleaching action and to hasten or promote such action heat has usually been applied, but it is often the case with this process that great difficulty has been experienced in obtaining 30 satisfactory colors by the use of such solutions.

When such difficulties arise, the use of excessive amounts of available chlorine has been resorted to in order to accomplish the 35 desired results, and in other cases—notably as set forth in the patents to Ornstein Nos. 1,298,553, and 1,298,554 and 1,298,555, it has been proposed to overcome the same objections by extreme dilution or by certain 40 actions which have never proved capable of very extended practicable or commercial application, being somewhat theoretical in character. It is believed from the results of experimental investigation of the processes 45 set forth in these patents, that economies in operation by their use can only be secured when small amounts of chlorine are required to bleach such fibres as rags, or old bleached paper. In the case of sulphite wood pulp,

esparto, hemp or soda wood pulp no appreciable advantages are to be gained by their use.

Another method adopted to speed up the bleaching action and secure greater economy in the process has been to use alum in the 55 bleaching vat. This, however, while a widely used plan and entirely successful in its ultimate results, is expensive and difficult to control, besides which it leaves aluminium oxide in the finished paper.

Another plan looking to the accomplishment of the same results has been to add sulfuric acid to the vat in addition to the calcium hypochlorite. This produces a violent reaction or effect and is, moreover, liable to injure the stock by rendering it tender, or by burning, besides which it releases free chlorine.

Still other methods that have been attempted or proposed for securing the desired results are set forth in the British Patent No. 11,333 of 1884, which involves the use of acetic acid; a successful but expensive proceeding, and also in British Patent No. 595 of 1883, which contemplates the 75 continued use of calcium hypochlorite and carbon dioxide, a plan involving great difficulty.

In an application filed by Wallace and Baker on April 24, 1920, Serial No. 376,224, 80 is described a process of producing hypochlorite solution by the instantaneous and continuous admixture of a solution of a base with chlorine, and in a series of experiments with this process of making bleaching solutions I discovered that if a larger proportion of chlorine were added to the basic solution than was required for the production of a neutral solution, a very rapid acting but unstable bleaching agent was the result. 85 I found in these experiments, however, that because of the presence of impurities from the base, in case lime were used, which had to be settled out before use, and by reason of the instability of the solution, it was 90 not practicable to economically use the process with lime.

I then discovered that if neutral or slight-

ly alkaline stable solutions were first prepared, settled and the clear liquor passed through the apparatus with the addition of chlorine gas equivalent in amount to approximately 5 to 10 per cent of the available chlorine in the solution, solutions were produced which, if used immediately, contained all of the original chlorine as well as that added, and that they possessed remarkable bleaching properties; that the process of bleaching was much more rapid than before; that the final colors obtained were much whiter than those produced by neutral solutions alone, and that less bleach was required to produce a given effect.

The promising nature of these results led to further investigation and experiment from which I have found that identical results could be obtained by the use of two separate solutions in the preparation of the bleach, one a neutral or slightly alkaline solution of hypochlorite, and the other a solution of chlorine water, and in this respects broadly the completed and most practicable embodiment of my present invention.

In carrying out this process for bleaching purposes, the hypochlorite solution in 1½ per cent to 4 per cent concentration is added to the pulp to be bleached and either simultaneously or after its introduction into the vat the desired amount of chlorine water is added to the pulp. At any practicable temperature this method of bleaching is preferable to that involving the use of neutral or alkaline hypochlorite solutions, but even better results are secured at the somewhat higher temperatures of 100° and 110° F.

The presence in the bleach of the additional chlorine may be obtained in either of two ways: First, chlorine gas may be added to a settled solution of hypochlorite by instantaneous contact such as practiced in the process of the Wallace and Baker application above referred to, but in this case the resulting solution must be used immediately for bleaching. Second, an aqueous solution of chlorine water may be combined with the solution of hypochlorite.

These two solutions may be produced in any known and preferred manner and are used either by admixture with each other in the required amounts to give the desired ratio between the two forms of chlorine, and used immediately after mixing, or the two solutions may be passed simultaneously into the bleaching vat, or finally the two solutions may be passed into the vat successively.

The first described method of introducing the chlorine gas with the hypochlorite solution has the advantage that it requires the minimum amount of dilution of the pulp in order to obtain the bleach. The second

method which involves the use of the two solutions, has a disadvantage in that it requires a larger volume or dilution than the first but it has the compensating advantage that the proportions of the agents may be much more readily varied as needed, and also that the solutions are both relatively stable before they are brought together. This greatly simplifies the plant control of the operation.

The reactions that occur in this process may be thus stated:



In the reactions as above written the amounts of each constituent required are not indicated, as this depends upon the concentration of the hypochlorite, the amount of lime in excess, the temperature, and the desired amount of hypochlorous acid in the final solution.

All variations desired in the bleaching may be controlled by the relative amount of chlorine added. The most important factor is the amount of HOCl in the solution, as in bleaching the results are largely due to this agent, which, however, should be present in the minimum amount to yield the desired color, speed and economy of operation.

As the bleaching proceeds the reactions which occur are:



Thus as rapidly as HOCl is consumed more is produced by the action of the formed HCl on the CaOCl<sub>2</sub> in solution. Such a bleaching solution as this, therefore, serves as a reservoir of hypochlorous acid keeping always a small, but constant, amount present during the bleaching. The presence of large amounts of this acid is to be avoided as other reactions occur with the materials described, rendering them difficult to bleach.

Having now described my invention what I claim is:—

1. A bleaching solution which consists of a solution of a base containing chlorine to an amount in excess of that required for neutralizing the same.
2. A bleaching solution consisting of a neutral hypochlorite solution containing an excess of chlorine.
3. A bleaching solution consisting of a neutral hypochlorite solution containing an excess of chlorine to the amount of ten per cent of the available chlorine in the solution.
4. The method of bleaching herein described which consists in introducing into the bleaching vat a neutral hypochlorite

solution and an excess of chlorine over that available in the solution.

5. The method of bleaching herein described which consists in introducing into the bleaching vat a neutral hypochlorite solution and a solution of chlorine in water.
6. The method of bleaching herein de-
- scribed which consists in simultaneously introducing and mixing in the bleaching vat a neutral hypochlorite solution, and a solution of chlorine and water. 10

In testimony whereof I hereto affix my signature.

JOHN C. BAKER.